

# UNITED STATES PATENT OFFICE.

DUNCAN McLEAN, OF WALLACETOWN, ONTARIO, CANADA.

## ROOF OR WALL COVERING.

SPECIFICATION forming part of Letters Patent No. 268,260, dated November 28, 1882.

Application filed April 15, 1882. (No specimens.)

*To all whom it may concern:*

Be it known that I, DUNCAN McLEAN, of Wallacetown, in the Province of Ontario and Dominion of Canada, have invented a new and Improved Roof or Wall Covering, of which the following is a full, clear, and exact description.

My improved composition of matter consists of the following ingredients, mixed in the following proportions, to wit: hydraulic cement, one barrel; clear sand, three barrels; salt, one-half bushel; hair and water in sufficient quantities to form a good mortar of medium stiffness. The salt is dissolved in the water, and the cement and sand are then mixed with the water to form a mortar, and the hair is added. This mortar is spread by means of a trowel to the thickness of about half an inch or more upon the roof, which must be covered with narrow lumber fastened on the roof with the joints not too close, so that some of the mortar can pass into the joints. Then one or more coats of hot gas or coal tar are applied by means of a brush, and as much sand is spread on this coal-tar as it will absorb and hold. This sanded surface is rubbed down smooth

by means of a suitable tool, upon which one or more coats of hot coal or gas tar are applied, and clear sand is spread on each coat of tar. When the coating is thoroughly dry and hard 30 it is rubbed with a suitable tool until it is smooth, hard, and glossy. Linseed-oil is to be used in this last operation to give the coating a good finish. This coating can be applied on the sides of a building in the same manner, 35 and can be painted any desired color.

This coating is water-proof, fire-proof, and frost-proof, is durable, and can easily be repaired, and is not very expensive.

Having thus described my invention, I claim 40 as new and desire to secure by Letters Patent—

A method of forming a roof or wall covering, which consists in first applying a coat of mortar on a slat frame, then covering this with alternate layers of gas or coal tar and sand, 45 and finally oiling as well as smoothing the outer surface, as described.

DUNCAN McLEAN.

Witnesses:

H. STANTON,  
HENRY S. ELLIS.